

April 27, 1926.

1,582,563

T. F. VON HAIMBERGER ET AL

METHOD OF COATING THE INNER SURFACES OF TUBES

Filed July 20, 1922



Inventors  
T. F. von Haimberger  
J. K. Wirth  
by Langmuir, Parry, Ward & Langmuir  
Atty's

## UNITED STATES PATENT OFFICE.

THEODOR FREIHEER VON HAIMBERGER, OF GRUNEWALD, NEAR BERLIN, AND  
JOHANN KARL WIRTH, OF CHARLOTTENBURG, NEAR BERLIN, GERMANY.

## METHOD OF COATING THE INNER SURFACES OF TUBES.

Application filed July 20, 1922. Serial No. 576,376.

To all whom it may concern:

Be it known that we, THEODOR FREIHEER VON HAIMBERGER and JOHANN KARL WIRTH, citizens of the German Republic, residing at 5 Grunewald, near Berlin, Germany, and Charlottenburg, near Berlin, Germany, have invented certain new and useful Improvements in Methods of Coating the Inner Surfaces of Tubes, of which the following is a 10 specification.

The present invention relates to a method of and apparatus for producing insulating coatings or coatings capable of offering resistance on the inner walls of tubes of metal, 15 metal fabrics or other materials. Such coatings may be produced for example by moistening the surface to be protected firstly with a phenol-formaldehyde condensation product serving as an adhesive and then 20 covering with a porous fibrous layer of asbestos or the like and then impregnating the layer and further treating in a suitable manner with a similar condensation product.

25 The employment of this mode of coating tubes offers considerable difficulties. Within the tube to be coated which is moistened with adhesive must be formed a new tube of fibrous material which tube must adhere 30 closely to the adhesive-coated wall of the outer tube while the adhesive must not be washed away, rubbed off or otherwise removed. These difficulties are still further increased by the fact that in the formation 35 of the coating of fibre pulp or the like generally a portion of the liquid from the pulp is pressed out and this liquid must be led off without damaging the adhesive layer below. Moreover, care must be taken to 40 avoid the formation of spaces between the tube and the covering layer.

Apparatus for performance of the method is illustrated in the accompanying drawing.

The apparatus serving in accordance with 45 this invention for producing coatings includes a supply pipe C which may either be stationary or may be rotated about its own axis and connected with the feed hopper A. This pipe may be smooth but may—if it is 50 to be rotated—be provided with worm-like projections. Into the pipe C extends a mandrel F which may either be stationary or may rotate about the longitudinal axis of the pipe C, said mandrel being provided if

desired at the end with worm-like projections and draining passages. A cover or stuffing box E is connected with the tube D to be coated by a screw thread or other easily detachable form of connection, the stuffing box being formed at X with small 60 air passages or holes. A braking device in the form of a weight, spring or friction producing device or the like (indicated diagrammatically in the drawing by a weight G connected with the cover) is provided. 65

For rotating the mandrel F, there is a gearing O, driven by the intermediary of any suitable means (not shown) and a movable support H slideable on a bed K or the like, for corresponding to the longitudinal 70 movement of the tube D on the mandrel F.

The modus operandi of the apparatus is as follows:—The adhesive liquid is applied to the tube D to be coated on the inside and to the supply pipe C on the outside 75 whereupon the tube D is pushed over the pipe C. By applying adhesive liquid to the supply pipe C the danger of removal of the adhesive layer in sliding the tube D over the pipe C is avoided. If desired, 80 during the pressing operation, adhesive liquid may be supplied to the space between the tubes D and C from Y.

The tube D to be coated is now closed by the cover E, and the mandrel F is brought 85 into the correct position and either secured or set in rotation about its longitudinal axis which coincides with the longitudinal axis of the supply pipe C.

Moist asbestos pulp or the like from the 90 feed hopper A is forced by means of the conveying worm B or by other suitable device through the supply pipe C against the mandrel F. The cover E takes the pressure. The braking device, shown in the drawing 95 by way of example, or another suitable braking device offers resistance to the movement of the tube D along the supply pipe C and the mandrel F. The fibre pulp or the like is now forced or pushed into the space 100 Z between the point of the mandrel and the pipe C until sufficient cohesion of the fibres and firm adhesion to the walls of the tube D is attained. Usually a portion of the liquid from the fibre pulp is pressed out. This 105 liquid may be led off through small channels at the end of the mandrel and can be drawn through a collector in the centre of the man-

drel. During the positive forward motion of the tube D the whole internal wall is covered homogeneously with the layer formed from the fibre pulp without damaging the layer of adhesive.

After these operations the tube is subjected to its further treatment.

In the performance of the method there may be used as an adhesive and impregnating medium, in addition to the condensation products of phenol and formaldehyde, other suitable materials, for example water-glass solutions, solutions of natural and artificial resins, solutions of celluloid, acetylcellulose, caoutchouc etc. To produce the coating there may be used in addition to fibrous materials, granular materials as for example quartz sand not too fine, fire-clay powder and so on. In this case the liquid of the pulp is preferably treated with some binding medium in order that after drying the inner layer produced will still remain porous but will hold together sufficiently so as not to break up during the subsequent impregnation.

What we claim is:—

1. A method of coating tubes with resisting substances, comprising, first coating a tube with a layer of adhesive material, then putting the coated tube telescopically over a supply conduit and a mandrel, then pressing a fibrous covering material through the supply conduit and into the hollow space between tube and mandrel to thereby slide the tube longitudinally over the mandrel, and supplying a resistance to the sliding of the tube.

2. A method of coating tubes with resisting substances, comprising, first coating a tube with a layer of adhesive material, then putting the coated tube telescopically over a supply conduit and a mandrel, then pressing a fibrous covering material through the supply conduit and into the hollow space between tube and mandrel to thereby slide the tube longitudinally over the mandrel supplying a resistance to the sliding of the

tube, and permitting the escape of liquid from the fibrous covering material.

3. A method of coating tubes with resisting substances, comprising, first coating a tube with a layer of adhesive material, then putting the coated tube telescopically over a supply conduit and a rotating mandrel, then pressing a fibrous covering material through the supply conduit and into the hollow space between tube and mandrel to thereby slide the tube longitudinally over the mandrel, and supplying a resistance to the sliding of the tube.

4. Apparatus for coating the inner wall of tubes, comprising a feed hopper for feeding the covering material, a supply conduit connecting with said feed hopper, a pointed end mandrel positioned in the longitudinal axis of the supply conduit and extending into the same with its pointed end, a slidable stuffing box positioned on the mandrel and braking means for regulating movement of the stuffing box relative to the said supply conduit.

5. Apparatus according to claim 4 said stuffing box being adapted to receive one end of a tube to be coated, and the supply conduit to receive the other end of the tube to be coated.

6. Apparatus according to claim 4 there being drain passages between the said mandrel and stuffing box.

7. A method of coating the inner wall of adhesive coated tubes with a covering material adapted to be attached thereto by means of the adhesive, comprising, applying an adhesive to the inner wall of a tube, pressing the covering material through a supply conduit sleeved by the adhesive-coated tube against a mandrel, thereby forcing said tube forward by the pressure of the covering material passing between the mandrel and the tube against a resistance.

In testimony whereof we affix our signatures.

Dipd. Ing. THEODOR FREIHERR von HAIMBERGER.

Dipd. Ing. JOH. KARL WIRTH.